# EUROPEAN PATENT SPECIFICATION

(11) **EP 0 048 929 B1**
(45) Date of publication and mention of the grant of the patent: **09.12.1987**
(21) Application number: 81107517.5
(22) Date of filing: 22.09.1981
(51) Int. Cl.: C25D 3/52, C25D 11/34, C25D 5/48

(54) **Rhodium-plated article with black or blue color, process for making the same and bath therefor**
Mit Rhodium einer schwarzen oder blauen Farbe bekleideter Gegenstand, Verfahren zu dessen Herstellung und Bad dafür
Article revêtu de rhodium de couleur noire ou bleue, procédé pour le fabriquer et bain utilisé dans ledit procédé

(30) Priority: 25.09.1980 JP 134038/80; 25.09.1980 JP 134039/80; 25.09.1980 JP 134040/80; 30.03.1981 JP 45522/81
(43) Date of publication of application: 07.04.1982
(62) Divisional of application: 85111660.8
(73) Proprietor: NIPPON MINING COMPANY LIMITED, Minato-ku Tokyo (JP); NIPPON METAL PLATING CO., LTD, Koto-ku TOKYO (JP)
(72) Inventor: Kinase, Takashi, Hitachi-shi, Ibaraki-ken (JP); Ichimura, Seiji, Katsuta-shi, Ibaraki-ken (JP); Mashiko, Masayoshi, Setagaya-ku, Tokyo (JP); Kinjo, Yoshio, Narashino-shi, Chiba-ken (JP); Matsumoto, Yosuke, CHiba-shi, Chiba-ken (JP); Suzuki, Kejiro, Hitachi-shi, Ibaraki-ken (JP)
(74) Representative: UEXKÜLL & STOLBERG

## Description

The present invention relates to a novel process and a novel rhodium-plating bath for producing a rhodium-plated article with black or blue colour.

Practically all the colors of the platings which are obtainable through known rhodium-plating baths are white, the known rhodium baths comprising various rhodium salts, e.g., sulfate or phosphate.

From FR-A-793 197 it is known to produce a black rhodium-plated article by electrodeposition from an acidic rhodium-plating bath containing additives like gelatine (Example 3) and benzoic acid (Example 1).

FR-A-2 427 404 relates to the electrodeposition of rhodium at a pH of 0.1 to 2.0 from a bath containing a rhodium salt and an inorganic (e.g. orthophosphoric) acid, to which an aminopolycarboxylic acid is added.

In US-A-3 592 750 the electroplating of titanium with a platinum group metal from a bath comprising an additive chosen from a variety of compounds including gelatine or non-aromatic sulfonates is disclosed.

Rhodium-plating has been generally employed for use in electric contacts, lead frames and ornamental articles due to its good hardness, wear resistance, corrosion or erosion resistance and stability in the contact resistance. Furthermore, it has been desired to develop rhodium plating with different colors besides white, as it will enhance the practical value of the rhodium plating.

On the other hand, known manners for black plating or black coloring such as black chrome plating, black nickel plating, blackening with copper carbonate all encounter difficulties in obtaining gloss, some of them yielding clouding, that is to say, these all being less valuable in the ornamental effect. There have been further problems in the manufacturing process, wherein they showed bad reproducibility in operation conditions, difficulties in mass production or the like. Thus there has been much to be desired in the prior art and it has long been desired to develop black color plating of noble metal in the ornamental article industries.

Accordingly, an object of the present invention is to provide a process and a plating bath for making a noble rhodium-plated article with black or blue color as well as mirror-like gloss.

Further objects of the invention will become apparent from the disclosure hereinbelow.

The inventors have become aware of the following fact after investigations for developing a bath composition for plating ("plating bath" or "bath" hereinafter) which provides a plating suitable for ornamental articles, particularly glasses, watches, accessories, cosmetics or dinner wares; rhodium-plating with black or blue color and mirror-like gloss is obtainable through a normal plating manner in an acid rhodium-plating bath comprising an additive selected from the group consisting ofthiomalic acid and salts thereof, phthalic acid and salts thereof, ethylenediamine, triethanolamine, sulfuric hydroxylamine, diethylenetriamine, butynediol and hypophosphite, the resultant rhodium-plating providing good adhesion and good corrosion or erosion resistance. Based on such finding, the inventors have completed the present invention.

The rhodium-plated articles of the present invention are suitable for, e.g., frames or glasses, cases, faces and bands of watches, necktie pins, lighters, necklaces, rings, compacts, caps for lipsticks and the like. The articles of the present invention may be utilized not only in the ornamental purpose but in various fields which require such a good plated coating.

The present invention will be described hereinbelow with reference to preferred embodiments which will, however, serve to better illustration of the invention and not to limitation thereof. Modifications may be done without aparting from the gist of the present invention.

The plating bath of the present invention comprises a normal acid rhodium plating bath comprising rhodium salt and free acid (known per se), and an additive consisting of at least one selected from the group consisting of thiomalic acid and salts thereof, phthalic acid and salts thereof, ethylenediamine, triethanolamine, sulfuric hydroxylamine, diethylenetriamine, butynediol and hypophosphite (referred to "additive" hereinafter). This plating bath is used for plating treatment of the articles resulting in rhodium-plated articles with desired properties.

Normally, the plating bath comprising three ingredients of rhodium salt, free acid and the additive will be sufficient for accomplishing the purpose of the present invention.

Rhodium salts which are normally used in the conventional rhodium plating, e.g., sulfate, phosphate, sulfamic acid and the like are employed as the rhodium salt for the plating bath.

The rhodium salt concentration in the bath ranges within a conventional, normal concentration, i.e., from 0.1 g/I to 20 g/l. At a concentration below 0.1 g/I the speed of electrodeposition will be undesirably reduced. At a concentration exceeding 20 g/I the expensive rhodium would be used without effective utilization.

The free acid encompasses acids which are normally used in the acid plating bath, such as sulfuric acid, phosphoric acid, sulfamic acid and the like.

Among the additives of the invention, thiomalic acid and phthalic acid are used in either a free acid form or a salt form, only one of these being sufficient, however, two or more being applicable. The terms thiomalic acid or phthalic acid denote also their salts hereinafter. Such salts encompass sodium or potassium salt.

The concentration of thiomalic acid and/or phthalic acid should be determined relating to the concentration of rhodium, and, however, be not less than 0.01 g/I, a lower concentration of which would deterioratingly affect upon color development. These additives may be added to the bath up to a solubility limit in the bath, however, used at a concentration which is practically sufficient.

The additives to the bath in the present invention further encompasses ethylenediamine, triethanolamine, sulfuric hydroxylamine, diethylenetriamine and butynediol. One amine among those as the additive is sufficient, however, two or more amines or amine(s) with other additives may be used.

The concentration of amine and butynediol in the bath approximates to that of the above-mentioned acids.

Hypophosphite as the additive encompasses alkali metal salts (sodium or potassium salt), alkaline earth metal salts (calcium or magnesium salt), other divalent metal salts (Co-, Ni-, Fe-, or Mn- salt) and the like. Among those salts alkali metal salts or alkaline earth metal salts are preferred.

The concentration of hypophosphite as the additive in the bath approximately ranges from 0.5 to 10 g/I. A lower concentration less than 0.5 g/I does not develop sufficient effect, and that exceeding 10 g/I would cause to get cloudy, i.e., to lose the gloss. This additive of hypophosphite requires slightly different conditions of plating with respect to pH, bath temperature or the like from the other additives aforementioned. For hypophosphite the pH should be below 2.5 as a higher pH would cause cracks or precipitation in the bath. An optimum temperature for hypophosphite approximately ranges from 20 to 45°C. A higher temperature exceeding 45°C is not preferred as it enhances the possibility of the partial clouding. However, the current density at a conventional, normal range (e.g., approximately 0.5-5 A/dm²) may be adopted.

The additives as hereinabove mentioned belong to essential ingredients of the bath according to the present invention, however, a further agent as a brightener may be added to the bath, i.e., 0.1-10 mg/I or nonionic surfactant may be used. Such nonionic surfactant encompasses that of the ether type, e.g. polyoxyethylenealkylether, polyoxyethylenealkylphenylether or the like, which are generally used as the brightener in the prior art, however, further serve to inhibit the plating from forming microcracks, partial clouding and to produce a uniform color tone.

Again turning to the additives of the invention other than hypophosphite, the pH value of the bath should not exceed 6. At a higher pH value than 6, rhodium in the bath will form hydroxide to form precipitation to disadvantage.

The color of the rhodium-plated coating or film relates to the thickness thereof, wherein a thinner coating will produce blue color while a thicker coating black color.

In the practical operation, it is also affected by plating conditions, whether the plating becomes black or blue, the plating conditions encompassing concentrations in the bath of the rhodium salt and the additive(s), bath temperature, current density, plating time, and the like. Such factors should be determined through a preparatory test plating under consideration of such factors. In the practical plating procedure, the control or choice of the color is preferably made mainly by changing the plating time under a predetermined bath condition.

The bath temperature and current density for plating procedure are adopted within the values as adopted in the conventional manner. A bath temperature of 10-80⁰C should be adopted. At a lower temperature less than 10°C, the current density will not sufficiently rise resulting in the low electrodeposition efficiency. At a temperature higher than 80°C, the disadvantage of violent vaporization of the bath will overcome the advantage of enhancement in the electrodeposition efficiency. The current density having close relation with the color tone should be 0.1-10 A/dm². A higher current density than 10 A/dm² will cause violent evaporation of gas at a cathode in the bath accompanied by a deteriorated color tone.

Materials for anode and cathode which are employed upon rhodium plating in the prior art may be used. The cathode may be selected from known material having a metallic surface such as brass, German silver (nickel silver), stainless steel or the like (however, iron, aluminium and zinc cannot be plated directly thereon). The cathode material further encompasses articles coated with strike (substrate coating), e.g., nickel strike or paradium-nickel strike. The cathode material encompasses also non-metallic articles coated with such substrate coating.

One of insoluble electrodes is sufficient for the anode, e.g., platinum electrode, titanium electrode coated with platinum or platinum-rhodium plating.

Other known manner generally applicable to the plating process may be optionally applied in the plating procedure in the present invention.

The article thus obtainable according to the present invention, however, has the mirror-like gloss with its surface, the black or blue color, good adhesion, good corrosion or erosion resistance, and the hardness compatible with the conventional rhodium plated articles without applying other conventional agents for various purposes. In other words, the rhodium-plated article with the black or blue color is obtainable through applying a bath essentially consisting of three ingredients, i.e., rhodium salt, free acid and the additive of the invention.

Thus the present invention is applicable in the industries with advantage.

Now, in the followings, the present invention will be described in more detail, by way of preferred embodiments thereof, which will not serve to limitation of the invention.

### Example 1

In a bath of pH 4.0 obtained by mixing rhodium sulfate (rhodium: 4 g/1), phthalic acid (2 g/1) and sulfuric acid were set_a titanium anode plated with platinum and a cathode of a brass watch case plated with a nickel strike.

The watch case was electroplated for ten minutes under conditions of a bath temperature of 30°C and a current density of 0.5 A/dm².

The resultant plating film presented black color and mirror-like gloss provided with 0.3 micron thickness and good adhesion.

The same article was electroplated for one minute under the same conditions. The resultant plating film was 0.03 micron thick provided with mirror-like gloss and blue color.

The resultant watch case was tested with respect to the corrosion resistance through a CAS-testing manner and exposure testing in an ammonia atmosphere. No corrosion was observed thus exhibiting the good corrosion resistance. The articles showed a hardness compatible with the level of the rhodium-plated white coating according to the conventional manner.
^{*}N.B. exposure in the ammonia atmosphere:
Sample pieces were put in a desiccator, charged with ammonia water of the density 0.96 on the bottom, the sample pieces were kept therein at 20°C for 24 hours exposed to an ammonia atmosphere. After the exposure, color change and bulging on the surface were observed.

### Examples 2-3

Rhodium-plating was carried out under the conditions as shown in Table 1 otherwise in the same condition as disclosed in Example 1, the results being also disclosed in Table 1. All the sample pieces showed properties equivalent to those of Example 1 with respect to the mirror-like gloss, corrosion resistance, hardness and adhesion.

### Example 4

Electroplating with rhodium was carried out under the conditions as shown in Table 2 otherwise under the same condition as in Example 1. The resultant plating film was 0.1 micron thick having good adhesion.

The good corrosion resistance was exhibited through the same testing as in Example 1, and the hardness compatible with the conventional white rhodium plating was exhibited.

By electroplating for 4 minutes otherwise under the same conditions as above, the resultant plating developed blue color provided with the thickness of 0.02 micron and other good properties as in the black rhodium plating.

### Examples 5-9

Rhodium plating was carried out under conditions as shown in Table 2 otherwise under the same conditions as in Example 1, the results being also disclosed in Table 2. The resultant platings showed the mirror-like gloss, the good corrosion-resistance and hardness as in Example 4.

## Claims

1. A process for producing a rhodium-plated article with black or blue colour which comprises
1) providing an acidic rhodium-plating bath comprised of rhodium salt, a free acid and at least one additive selected from thiomalic acid and salts thereof, phthalic acid and salts thereof, ethylenediamine, triethanolamine, sulfuric hydroxylamine, diethylenetriamine, butynediol and hypophosphite, said additive being present in an amount of at least 0.01 g/I, with the pH of said bath not exceeding 6; and
2) electroplating an article in said rhodium-plating bath under conditions such that the rhodium-plating film develops black or blue colour.

2. An acidic rhodium-plating bath for producing a rhodium-plated article with black or blue colour comprised of rhodium salt, a free acid and at least one additive selected from thiomalic acid and salts thereof, phthalic acid and salts thereof, ethylenediamine, triethanolamine, sulfuric hydroxylamine, diethylenetriamine, butynediol and hypophosphite, said additive being present in an amount of at least 0.01 g/I, with the pH of said bath not exceeding 6.

3. The process according to claim 1 or the rhodium-plating bath according to claim 2, wherein said hypophosphite is selected from an alkali metal salt, an alkaline earth metal salt, a divalent metal salt other than alkaline earth metal salt, or mixtures thereof.

4. The process according to claim 1 or the rhodium-plating bath according to claim 2, wherein said additive is hypophosphite and the pH value of the bath does not exceed 2.5.

5. The process or the rhodium-plating bath according to any of claims 1 to 4, wherein said free acid is selected from sulfuric acid, phosphoric acid and sulfamic acid.

## Patentansprüche

1. Verfahren zur Herstellung eines rhodium-plattierten Gegenstands mit schwarzer oder blauer Farbe, dadurch gekennzeichnet, daß
1) ein saures Rhodium-Plattierungsbad zur Verfügung gestellt wird, daß Rhodiumsalz, eine freie Säure und mindestens ein Additiv ausgewählt aus Thioäpfelsäure und Salzen derselben, Phthalsäure und Salzen derselben, Ethylendiamin, Triethanolamine, schwefelsaures Hydroxylamin, Diethylentriamin, Butindiol und Hypophosphit umfaßt, wobei das Additiv in einer Menge von mindestens 0,01 g/l vorhanden ist und der pH-Wert des Bades 6 nicht übersteigt und
2) ein Gegenstand in diesem Rhodium-Plattierungsbad unter solchen Bedingungen elektroplattiert wird, daß der Rhodiumplattierungsfilm eine schwarze oder blaue Farbe entwickelt.

2. Saures Rhodium-Plattierungsbad zur Herstellung eines Rhodium-plattierten Gegenstands mit schwarzer oder blauer Farbe, gekennzeichnet durch Rhodiumsalz, eine freie Säure und mindestens ein Additiv ausgewählt aus Thioäpfelsäure und Salzen derselben, Phthalsäure und Salzen derselben, Ethylendiamin, Triethanolamin, schwefelsaures Hydroxylamin, Diethylentriamin, Butindiol und Hypophosphit umfaßt, wobei das Additiv in einer Menge von mindestens 0,01 g/I vorhanden ist und der pH-Wert des Bades 6 nicht übersteigt.

3. Verfahren nach Anspruch 1 oder Rhodium-Plattierungsbad nach Anspruch 2, dadurch gekennzeichnet, daß das Hypophosphit ausgewählt ist aus einem Alkalimetallsalz, einem Erdalkalimetallsalz, einem Salz eines anderen zweiwertigen Metalls als dem eines Erdalkalimetalls oder Mischungen derselben.

4. Verfahren nach Anspruch 1 oder Rhodium-Plattierungsbad nach Anspruch 2, dadurch gekennzeichnet, daß das Additiv Hypophosphit ist und der pH-Wert des Bades 2,5 nicht übersteigt.

5. Verfahren oder Rhodium-Plattierungsbad nach einem der Ansprüche 1 bis 4, dadurch gekennzeichnet, daß die freie Säure ausgewählt ist aus Schwefelsäure, Phosphorsäure und Sulfamidsäure.

## Revendications

1. Procédé de production d'un article avec un placage de rhodium ayant une couleur noire ou bleue, qui consiste
1) à préparer un bain acide de placage de rhodium comprenant un sel de rhodium, un acide libre et au moins un additif choisi entre l'acide thiomalique et ses sels, l'acide phtalique et ses sels, l'éthylènediamine, la triéthanolamine, l'hydroxylamine sulfurique, la diéthylènetriamine, le butynediol et un hypophosphite, ledit additif étant présent en une quantité d'au moins 0,01 g/I, le pH du bain ne dépassant pas 6; et
2) à soumettre un article à une électrodéposition dans le bain de placage de rhodium dans des conditions choisies de manière que le placage de rhodium développe une coloration noire ou bleue.

2. Bain acide de placage de rhodium pour la production d'un article avec un placage de rhodium ayant une couleur noire ou bleue, comprenant un sel de rhodium, un acide libre et au moins un additif choisi entre l'acide thiomalique et ses sels, l'acide phtalique et ses sels, l'éthylènediamine, la triéthanolamine, l'hydroxylamine sulfurique, la diéthylènetriamine, le butynediol et un hypophosphite, ledit additif étant présent en une quantité d'au moins 0,01 g/I, le pH du bain ne dépassant pas 6.

3. Procédé suivant la revendication 1 ou bain de placage de rhodium suivant la revendication 2, dans lequel l'hypophosphite est choisi entre un sel de métal alcalin, un sel de métal alcalino-terreux, un sel de métal divalent autre qu'un sel de métal alcalino-terreux, ou leurs mélanges.

4. Procédé suivant la revendication 1 ou bain de placage de rhodium suivant la revendication 2, dans lequel l'additif est un hypophosphite et la valeur du pH du bain ne dépasse pas 2,5.

5. Procédé ou bain de placage de rhodium suivant l'une quelconque des revendications 1 à 4, dans lequel l'acide libre est choisi entre l'acide sulfurique, l'acide phosphorique et l'acide sulfamique.
